



US007879772B2

(12) **United States Patent**  
**Komiyama et al.**

(10) **Patent No.:** **US 7,879,772 B2**  
(45) **Date of Patent:** **Feb. 1, 2011**

(54) **PROCESS FOR COLD PLASTIC WORKING  
OF METALLIC MATERIALS**

(75) Inventors: **Shinobu Komiyama**, Tokyo (JP);  
**Masayuki Yoshida**, Tokyo (JP);  
**Hidehiro Yamaguchi**, Tokyo (JP)

(73) Assignee: **Nihon Parkerizing Co., Ltd.**, Tokyo  
(JP)

(\*) Notice: Subject to any disclaimer, the term of this  
patent is extended or adjusted under 35  
U.S.C. 154(b) by 123 days.

(21) Appl. No.: **12/382,215**

(22) Filed: **Mar. 11, 2009**

(65) **Prior Publication Data**

US 2009/0178454 A1 Jul. 16, 2009

**Related U.S. Application Data**

(62) Division of application No. 10/508,999, filed as application No. PCT/JP03/03511 on Mar. 24, 2003, now abandoned.

(30) **Foreign Application Priority Data**

Mar. 25, 2002 (JP) ..... 2002-083906

(51) **Int. Cl.**

**C10M 137/06** (2006.01)  
**C10M 129/40** (2006.01)  
**C23C 22/12** (2006.01)

(52) **U.S. Cl.** ..... **508/108; 427/435**

(58) **Field of Classification Search** ..... **508/108;  
427/435**

See application file for complete search history.

(56) **References Cited**

U.S. PATENT DOCUMENTS

|             |         |                     |
|-------------|---------|---------------------|
| 3,619,264 A | 11/1971 | Worms et al.        |
| 4,192,793 A | 3/1980  | Tanioka et al.      |
| 4,294,808 A | 10/1981 | Wasel-Nielen et al. |
| 4,461,680 A | 7/1984  | Lashmore            |
| 4,761,188 A | 8/1988  | Miyata              |
| 5,024,826 A | 6/1991  | Linton              |
| 5,039,408 A | 8/1991  | Ichitsuka et al.    |
| 5,211,833 A | 5/1993  | Shirkhanzadeh       |
| 5,480,480 A | 1/1996  | Lynch et al.        |

|                 |         |                             |
|-----------------|---------|-----------------------------|
| 5,587,059 A     | 12/1996 | Yamoto et al.               |
| 6,001,784 A     | 12/1999 | Trivett                     |
| 6,015,855 A     | 1/2000  | Dalton                      |
| 6,150,308 A *   | 11/2000 | Deruyck et al. .... 508/348 |
| 2001/0031693 A1 | 10/2001 | Hoke et al.                 |

FOREIGN PATENT DOCUMENTS

|    |                |         |
|----|----------------|---------|
| GB | 1257172 A      | 12/1971 |
| GB | 2257712 A      | 1/1993  |
| JP | 51-44579 A     | 4/1976  |
| JP | 52-20967       | 2/1977  |
| JP | 56-59896 A     | 5/1981  |
| JP | 58-15594 A     | 1/1983  |
| JP | 01110567 A *   | 4/1989  |
| JP | 6-346075 A     | 12/1994 |
| JP | 11100205 A     | 4/1999  |
| JP | 2000154010 A * | 6/2000  |
| WO | 97/48783 A1    | 12/1997 |
| WO | 99/64544 A1    | 12/1999 |

OTHER PUBLICATIONS

Supp. European Search Report in EP 03 72 0889 mailed Feb. 3, 2010.

\* cited by examiner

*Primary Examiner*—Glenn Calderola

*Assistant Examiner*—Jim Goloboy

(74) *Attorney, Agent, or Firm*—Nixon & Vanderhye P.C.

(57) **ABSTRACT**

Particles each of which consists of an inorganic polyvalent metal compound as a nucleus and a coating of a metallic soap of the polyvalent metal coating the nucleus (coated particles); products and preparation processes using the particles; a lubricating coating forming agent wherein particles each of which consists of a polyvalent metal salt of phosphoric acid as a nucleus and a coating of a metallic soap of the polyvalent metal coating the surface of the nucleus are suspended in an aqueous solution of a water soluble inorganic salt and/or a water soluble organic acid salt; and a lubricating coating. The coated particles are novel particles which can be used as an ingredient of coating-type lubricating coating; are excellent in seizure resistance; can inhibit wear of tools at the time of plastic working since the friction coefficient of the surface of the particles is low; and are slow to cause pollution of working oils. Lubricating coating obtained by applying the lubricating coating forming agent onto the surface of a metallic material gives excellent cold plastic working properties, namely lubricity and seizure resistance to the metallic material.

**19 Claims, No Drawings**

## 1

PROCESS FOR COLD PLASTIC WORKING  
OF METALLIC MATERIALS

This application is a divisional of application Ser. No. 10/508,999 filed Sep. 27, 2004 now abandoned, which in turn is the US national phase of international application PCT/JP03/03511 filed 24 Mar. 2003, which designated the US and claims benefit of JP Application No. 2002-83906 filed 25 Mar. 2002, the entire contents of each of which are incorporated herein by reference.

## TECHNICAL FIELD

This invention is roughly classified into two relevant inventions. One is an invention relating to particles of an inorganic polyvalent metal compound coated with a metallic soap as a fundamental invention, and their general utilization forms; and the other is an invention relating to a plastic working lubricant containing such coated particles as a more practical application form of such coated particles.

The invention as a fundamental invention can be used in a wide range, and relates to metallic soap-coated particles excellent in seizure resistance and capable of preventing tools from wear and working oil from pollution at the time of plastic working; powder or suspension on such particles; a process for preparing the powder or suspension; and lubricating coating.

The invention as a more practical applied invention relates to a lubricating coating forming agent, and, in more detail, relates to a lubricating coating forming agent giving excellent workability, namely excellent lubricity and excellent seizure resistance onto the surfaces of various metallic materials such as, for example, iron materials, steel materials, stainless steel materials, aluminum materials, magnesium materials, tin materials and titanium materials which need to be subjected to cold plastic working typically including forging, wire drawing, tube reducing and sheet forming; and lubricating coating.

## BACKGROUND ART

## Background Art Particularly About the Present Invention as a Fundamental Invention

Metallic soap widely used as various lubricants, etc. plays an important role in the field of cold plastic working typically including forging, wire drawing, tube drawing of pipes, sheet forming, etc. of metallic materials. In this field, metallic soap has been used from long ago as a lubricating ingredient to lower the friction coefficient between materials to be wrought and tools at the time of plastic working and thereby reduce working energy drastically, and has greatly contributed to development of the cold plastic working field. For example, as a direct use example of metallic soap in the plastic working field, there can be mentioned its utilization in auxiliary lubricants used at wire drawing working. This is such a technology that when a carrier layer such as borax coating, slaked lime coating or zinc phosphate coating is provided on the surface of a wire rod and the rod is subjected to wire drawing working, immediately before the material to be wrought passes through the die, an auxiliary lubricant containing a large amount of a metallic soap is made to adhere onto the material to give or supplement lubricity; and is a case where powder of the metallic soap is used in a large amount. In another case, a coating-type lubricant in which lubricating particles containing a metallic soap as a main ingredient are suspended in water or an oil, etc. are used in many combinations with the

## 2

above-mentioned carrier layer; and so on, and thus there are many technologies applying metallic soap in the cold plastic working field.

However, there are also problems in use of metallic soap. 5 As one of them, there can be mentioned a case of steel wire for header working in which wire a carrier layer is provided by lime-type coating forming treatment, an auxiliary lubricant containing a metallic soap as a main ingredient is made to adhere thereon, and lubricating coating is completed by carrying out skin pass wire drawing working. The resulting lubricating coating-coated steel wire is subjected to header working in a working oil, but at that time, the metallic soap in the lubricating coating scraps peeling off swells or is finely suspended in the working oil to pollute the working oil 10 extremely. This phenomenon is thought to occur because adhesion between the carrier layer and the lubricating coating layer is low.

On the other hand, as a lubricating coating forming technology, which is somewhat different from the above technol-

20 25 30 35

ogy directly using metallic soap, but is very interesting in using metallic soap and very fit for cold plastic working, "phosphating treatment plus soap treatment" has generally been used from long ago in this field. This technology is such that a phosphate salt coating layer is previously provided onto the surface of a material to be wrought, the coating layer firmly adhering to the surface as a reactive chemical conversion coating treatment layer, and then an aqueous solution of a water soluble fatty acid salt is contacted with the coating layer at an elevated temperature to form metallic soap coating containing a reactive soap layer. Since the phosphate salt coating surface is firmly coated with the metallic soap layer, this technology has such advantages in comparison with the above-mentioned "carrier layer plus auxiliary lubricant" that the technology is fit for comparatively strong working since working following properties of the lubricating ingredient are good, and such a phenomenon is hard to cause that the soap and the metallic soap are isolated from the lubricating coating scraps peeling off at the time of working and pollute the working oil extremely; and so on.

40 45 50

However, since both of the phosphating treatment and the coating treatment with the metallic soap onto the resulting layer are coating forming methods utilizing chemical reaction, control of the chemical reactions and administration activity at the cold plastic working site are complicated, and when waste water treatment and plant and equipment investment are included, vast costs are needed. Furthermore, since the performance of coating formed greatly varies depending on kinds of steels, surface states of steel, etc., labor for maintaining stable quality is very large, and, furthermore, mass formation of industrial wastes is coming to be a great anxiety on environmental load. Thus, in recent years, development of a convenient and ecological coating forming process has positively been attempted.

55 60 65

Lubricating coating comes in between the material to be wrought and the tool at the time of plastic working to avoid direct metal contact between the material to be wrought and the tool, and such lubricating coating may be liquid or solid. However practically, liquid lubricants represented by oil-type lubricants, etc. are often unfit for severe plastic working. The reason is that the lubricating coating preventing the material to be wrought and the tool from their direct contact undergoes shear to cause lubricating coating cutting, and thereby seizure occurs. Thus, even when a liquid lubricant is used or a lubricating ingredient such as metallic soap which melts and is liquidized with working heat is used, it is general to use it in combination with carrier coating such as phosphate salt coating or borax coating, and thereby, the lubricating ingredient

together with the carrier layer comes in between the surface of the material to be wrought and the tool at the time of working, and reduces working force and prevents seizure. But strictly speaking, since, even in this situation, lubrication coating cutting occurs between the carrier layer surface and the tool surface, there sometimes arises a situation that the tool surface undergoes wear little by little by the carrier layer having a high friction coefficient and the life of the tool gets short, which gets to be a problem.

Furthermore, recently, there is a tendency that by shortening the step of cold plastic working for the purpose of heightening productive efficiency, the degree of one working is heightened, and, even in "phosphating treatment plus soap treatment", it gets difficult to follow surface area enlargement with sufficient lubricating layer held.

As a technology for forming cold plastic working lubricating coating for solving these problems, a step shortening-type lubricating coating forming agent, etc. are being developed. This technology is one capable of giving high cold plastic working performance by simple steps only to make a liquid coating forming agent adhere onto the surface of a material to be wrought and dry the agent. As such an invention, JP 2000-63880 A discloses a lubricant composition for plastic working of metallic material which comprises (A) a synthetic resin, (B) a water soluble inorganic salt and water, (B)/(A) (ratio by weight in terms of solid matter) being 0.25/1 to 9/1, the synthetic resin dissolving or being dispersed. It is also disclosed that it is preferred to further incorporate as a lubricant ingredient at least one selected from the group consisting of a metallic soap, a wax, polytetrafluoroethylene and an oil in an amount of 1 to 20% by mass, and as the water soluble inorganic salt is preferred at least one selected from the group consisting of a sulfate, a borate, molybdate, a vanadate and a tungstate. Namely, this invention is characterized in that a lubricating ingredient such as a metallic soap or a wax is contained, in a dispersed state, in coating ingredients capable of becoming a carrier, and is an excellent technology capable of obtaining lubricating coating having high working performance simply and with labor saving only by applying the composition onto the surface of the material to be wrought. Although metallic soap is often used as the lubricating ingredient, it is mentioned that, since the metallic soap is immobilized in the coating by the inorganic salt and/or the resin ingredient, adhesion of the metallic soap is not influenced by adhesion between layers, as is the case in "carrier layer plus auxiliary lubricant layer", the possibility of peeling of the metallic soap alone at the time of working is generally small. Furthermore, in comparison with the coating of "phosphate salt plus soap treatment" which is lubricating coating consisting of a comparatively large size of crystals of the order of width 200  $\mu\text{m}$ , coating obtained from the above invention has an advantage that it is possible to adjust the surface area of the lubricant at will, e.g. by making lubricant ingredients fine particles, and thus lubricating coating exerting excellent performance even in strong working where enlargement of surface area is large is being developed, and the technology including the above invention is a prospective technology also in the aspect of lubricating performance. However, even in the case of the lubricating coating obtained by the above technology, there is a tendency that the carrier layer of a high friction coefficient exposed owing to the structure of the coating repeats contact with the tool to give the tool life bad influence.

Under such a present state of things, lubricating coating required in the cold plastic working field is considered to be lubricating coating which has such fine particle structure that the lubricant layer coats the carrier layer and strongly adheres

to the carrier layer, and can be obtained by coating-type treatment without needing complicated treating steps. By this, it gets possible to realize ecological treatment of shortened steps, reduction of loads on the tool (i.e., reduction of tool wear), reduction of pollution of the working oil by lubricating coating scraps, etc. Development of such an ideal lubricant is a great problem and is urgently needed.

Background Art Particularly About the Present Invention as a More Practical Applied Invention

In plastic working of metallic material, lubricating coating is formed on the surface of the material to be wrought, for preventing seizure and galling formed by direct metal contact between the material to be wrought and the tool. As lubricating coating formed on the surface of the material to be wrought, there are two types, one being lubricating coating formed by making a lubricant physically adhere to the surface of the material to be wrought, the other being lubricating coating formed by forming a chemical conversion coating on the surface of the material to be wrought through chemical reaction and then applying a lubricant.

Lubricants made to adhere onto the surface of the material to be wrought are inferior, in adhesion, to lubricants used after formation of a chemical conversion coating on the material to be wrought, and thus generally used in light working. In use of a chemical conversion coating, a chemical conversion coating such as a phosphate coating or an oxalate coating playing a role as a carrier is formed on the material to be wrought, and then a lubricant having good slipping properties is applied thereon. This type of coating has two layer structure consisting of the conversion coating as a carrier coating and the lubricant coating and exerts very high seizure resistance, and thus has very widely been used in the field of plastic working such as wire drawing, tube reducing and forging. Particularly in a field of severe working among the plastic working field, a method of using phosphate coating or oxalate coating as undercoat and applying a lubricant thereon is being frequently adopted.

Methods for forming a chemical conversion coating onto a material to be wrought and applying a lubricant thereon are classified broadly into two methods. One is a method of making a lubricant physically adhere onto the chemical conversion coating, and the other is a method of reacting a lubricant with the surface of the chemical conversion coating to form lubricating coating.

As the lubricant of the former made to physically adhere, there can be mentioned one obtained by adding an extreme pressure additive into mineral oil, vegetable oil or synthetic oil as a base oil; one obtained by dissolving or dispersing a solid lubricant represented by graphite or molybdenum disulfide together with a binder ingredient in water; etc. Such a lubricant is applied onto the surface of a material to be wrought which was subjected in advance to chemical conversion coating treatment, and, in the application, the oil lubricant is used as such, and the aqueous lubricant is used, followed by a drying step. These lubricants have advantages that there is no restriction about their application method and convenient spray coating or immersion coating can be used; and complicated liquid control as in chemical conversion coating treatment is almost unnecessary; etc., but these lubricants are often used in comparatively light working because of low lubricity.

On the other hand, as the lubricant of the latter to react it with the chemical conversion coating, there can generally be mentioned reactive soap. This method is a technology which has generally been used from long ago as "phosphating treat-

ment plus soap treatment", and according to the method, a chemical conversion coating is formed on the surface of material to be wrought, and then an aqueous solution of a water soluble fatty acid salt is contacted with the coating at elevated temperature to form, on the coating, metallic soap coating containing the reactive soap. The composite coating formed according to this method can be adapted to from light working to comparatively strong working, and is used in a very wide range of working including forging and tube reducing.

However, as to reactive-type chemical conversion coating treatment and reactive soap treatment, there are two problems in a broad classification. One is that treatment steps for chemical conversion coating treatment and soap treatment are complicated; that very wide space is needed as the treatment space; and that control of treating steps is very complicated, for example that control of the concentration and ingredients of the treating liquid, and temperature control for controlling the reaction are needed because these treatments utilize chemical reactions. The other is that the amount of industrial wastes and waste water is very large, for example that since insoluble salts generally called sludge are formed in the treating liquid as by-products of the reactions, it is necessary to discharge them periodically from the treating liquid, and that since when the treating liquid is used successively, the ingredient balance of the treating liquid is spoiled, disposal and renewal of the treating liquid, etc. get necessary.

Detailed explanation is made bellow on the former. When "phosphate treatment plus soap treatment" is taken up as an example, a material to be wrought is first subjected to the cleaning step and the descaling step, and then to phosphating treatment and soap treatment. Since single or multi-stage water washing steps are necessary among these steps, space of about 7 to 12 vessels gets necessary as treating vessel space. Furthermore, control of the concentration and temperature of the treating liquid is necessary on each of the treating steps, and, in the phosphating step, free acid degree, total acid degree and accelerator concentration in the treating liquid are measured by manual operation according to a neutralization titration method and the like, and insufficient ingredients are supplemented appropriately. Furthermore, as to temperature, there are plural steps where the treatment is made at 60 to 80°C. and the heating is carried out with steam piping or the like, and thus a large amount of energy is used.

Detailed explanation is made bellow on the latter. When steel or iron material to be wrought is subjected to phosphating treatment, the surface of the material is etched in the phosphating solution and iron ions are eluted into the solution. Transfer of electrons occurs by this reaction and phosphate salt coating is formed, but for acceleration of the reaction, it is needed to deposit and precipitate the iron ions as an insoluble salt. This insoluble salt is generally called sludge. The sludge needs to be periodically discharged from the system. Furthermore, water washings after the pretreatments prior to chemical conversion coating treatment and after the chemical conversion coating treatment are contaminated with the treating liquids of the previous steps, respectively. Since the respective washings contain various elements, appropriate waste water treatments get necessary. Usually, these washings as waste water are discharged after subjection to neutralization treatment, coagulating sedimentation treatment, etc., but coagulating sedimentation sludge containing phosphorus, etc. is dumped as industrial wastes as is the case with the above-mentioned sludge.

In recent years, reduction of industrial wastes has been aimed as a large problem for the protection of earthly environment. Among such activities, chemical conversion coating treatment forming a lot of industrial wastes as mentioned

above is taken up as one of large problems, and an alternative lubricant and/or an alternative treating system each forming less industrial wastes have/has strongly been desired.

For solving these problems, "a lubricating composition 5 wherein a water soluble macromolecule or an aqueous emulsion thereof is used as a base material and a solid lubricant and a chemical conversion coating forming agent are compounded" etc., are disclosed in JP 52-20967 A, but coating equal to coating from chemical conversion coating treatment 10 is not obtained. Also as a means for solving the above problems, there can, for example, be mentioned the invention of "an aqueous lubricant for cold plastic working of metallic material" disclosed in JP 10-8085 A and filed by the present applicant. The invention relates to an aqueous lubricant for 15 cold forging working of metal which comprises (A) a water soluble inorganic salt, (B) a solid lubricant, (C) a at least one oil ingredient selected from mineral oil, vegetable or animal oil and synthetic oil, (D) a surfactant and (E) water, and wherein the solid lubricant and the oil are uniformly dispersed and emulsified.

The invention relates to an aqueous non-reactive-type lubricant, and, therein, it is aimed to shorten the three steps of phosphating treatment-water washing-reactive-type soap treatment to one step of lubrication treatment alone. Namely, 25 the aqueous non-reactive-type lubricant is contacted with a cleaned material to be wrought by immersion or the like to coat the surface of the material with the lubricant, and then dried (evaporation of water) to form lubricating coating on the surface of the material. Such type of lubricant is called one-step lubricant. However, the lubricant of the above invention 30 is too unstable to be used industrially because it emulsifies an oil ingredient, and has not exerted stable lubricity in cold forging of large working degree or in tube drawing working where continuous heat load is imposed on the lubricating coating.

As a further means for solving the above-mentioned problems, there can, for example, be mentioned the invention of "a lubricant composition for plastic working of metallic material" disclosed in JP 2000-63880 A and made by the present 40 applicant. The invention relates to a lubricant composition for plastic working of metallic material which comprises (A) a synthetic resin, (B) a water soluble inorganic salt and water, and wherein the ratio by mass of (B)/(A) in terms of solid matter is 0.25/1 to 9/1 and the synthetic resin is dissolved or dispersed. However even in the invention, stable lubricity has 45 not been exerted in cold forging of large working degree or in tube drawing working where continuous heat load is imposed on the lubricating coating. Furthermore in the invention, stable lubricity has not been exerted either in the cases where 50 it is difficult, in actual operation, to apply a lubricant uniformly, for example in barrel treatment in cold forging, in bundled treatment in tube reducing working or in coil treatment in wire drawing working. Although it is indispensable to 55 solve the above problems in use of a coating-type lubricant, it is a present state of things that an effective solution has not yet been found.

#### DISCLOSURE OF INVENTION

##### Problem 1

The present invention is for solving problems which prior art (particularly prior art on the present invention as a fundamental invention) has, and aims to provide novel particles, as an ingredient used mainly in coating-type lubricating coating, which are excellent in seizure resistance, and can inhibit wear of tools at the time of plastic working due to a low friction

coefficient of their surfaces, and are slow to cause pollution of working oil; such particles that, when the particles are incorporated into a lubricant layer, the lubricant layer can make itself firmly composite with the carrier layer so that the former layer may coat the latter layer; powder consisting of the particles; a suspension containing the particles; processes for preparing the powder or suspension; and lubricating coating containing the particles.

#### Means for Solving Problem 1

The present inventors have intensely studied for solving the above problems (particularly Problem 1). As a result, they found that particles each of which consists of an inorganic polyvalent metal compound as a nucleus and a coating of a metallic soap of the polyvalent metal coating the nucleus, the inorganic polyvalent metal compound being water sparingly soluble or water insoluble and having reactivity with an alkali metal salt, ammonium salt or water soluble ester of a fatty acid; or particles each of which consists of each of the particles defined above and a coating of an alkali metal salt, ammonium salt or water soluble ester of a fatty acid coating the particle, when used mainly as an ingredient in coating-type lubricating coating, are very suitable as a material which is excellent in seizure resistance, can inhibit wear of tools at the time of plastic working due to a low friction coefficient of their surfaces, and is slow to cause pollution of working oil; and completed this invention.

Namely, the invention relates to particles each of which consists of an inorganic polyvalent metal compound as a nucleus and a coating of a metallic soap of the polyvalent metal coating the surface of the nucleus, the inorganic polyvalent metal compound being water sparingly soluble or water insoluble and having reactivity with an alkali metal salt, ammonium salt or water soluble ester of a fatty acid (hereinafter, the above particles are sometimes referred to as two-layer particles); particles each of which consists of each of the particles defined above and a coating of an alkali metal salt, ammonium salt or water soluble ester of a fatty acid (hereinafter, the “alkali metal salt, ammonium salt or water soluble ester of a fatty acid” is sometimes referred to as “alkali soap or the like”) coating the surface of the particle (hereinafter, the above particles are sometimes referred to as three-layer particles); powder consisting of the particles; a suspension wherein the above particles are suspended in water or an aqueous solution of an alkali soap or the like, the average particle size of particles of the inorganic polyvalent metal compound being 20  $\mu\text{m}$  or less, the proportion of all the metallic soap coatings to all the particles being 1 to 30% by mass; a process for preparing the above powder or suspension; lubricating coating containing the above particles in an amount of 1% by mass or more. Hereinafter, the two-layer particles and/or three-layer particles are sometimes referred to as coated particles.

#### Problem 2

The present invention is also for solving problems which prior art (particularly prior art on the present invention as a more practical applied invention) has. Namely, the invention aims to provide such a lubricating coating forming agent that protection of earthly environment is taken into consideration; convenient treatment by a spraying method or immersion method is possible; chemical conversion coating treatment is unnecessary; and resulting coating has excellent working performance and excellent seizure resistance equal to or more than those in chemical conversion coating treatment method,

and, even when uniform application is difficult as mentioned above, exerts stable lubricating properties owing to self-repairing effect.

#### Means for Solving Problem 2

The present invention have intensely studied for solving the above problems (particularly Problem 2), and as a result, they found that lubricating coating wherein cold forging working of large working degree is possible and which exerts good lubricity even in tube drawing working in which continuous heat load is imposed on the coating, can be obtained by a convenient treating method of applying, onto a material to be wrought, an aqueous solution containing particles each of which consists of a polyvalent metal salt of phosphoric acid as a nucleus and a coating of a metallic soap of the polyvalent metal coating the surface of the nucleus, and a water soluble inorganic salt and/or a water soluble organic acid salt, and drying the resulting wet coating; and further found that the above-mentioned particles have both seizure resistance and lubricity, and, therefore, even in a case as mentioned above where uniform coating is difficult, the particles are introduced into the tool by melted ingredients in the coating and exert self-repairing effect on the defect parts of the coating, and, finally, the coating exerts stable lubricity; and completed the present invention.

Namely, the invention relates to a lubricating coating forming agent wherein particles each of which consists of a water sparingly soluble or water insoluble polyvalent metal salt of phosphoric acid (hereinafter merely referred to as polyvalent metal salt of phosphoric acid) as a nucleus and a coating of a metallic soap of the polyvalent metal coating the surface of the nucleus (the particles being hereinafter referred to as particles of coated polyvalent metal salt of phosphoric acid) are suspended in an aqueous solution of a water soluble inorganic salt and/or a water soluble organic acid salt; each of the water soluble inorganic salt and organic acid salt having a property to form a firm coating when it is uniformly dissolved in water and the resulting solution is applied on a metallic material and dried.

The above particles of coated polyvalent metal salt of phosphoric acid are included in the above-mentioned “two-layer particles” in the present invention as a fundamental invention.

#### BEST MODE FOR CARRYING OUT THE INVENTION

The invention is described in detail below, and, first, the invention as a fundamental invention is mainly described in detail, and, then, the invention as a practical applied invention is mainly described in detail.

##### Detailed Description Particularly on the Invention as a Fundamental Invention

The inorganic polyvalent metal compound which is used for preparing the coated particles of the invention, and is water sparingly soluble or water insoluble and has reactivity with an alkali soap or the like is an important ingredient as a nucleus immobilizing the metallic soap layer in the coated particles of the invention. The inorganic polyvalent metal compound used in the invention is a granular substance usually supplied as powder or in a state dispersed in water. The inorganic polyvalent metal compound is not particularly limited, and includes oxides, hydroxides, carbonates, phosphates, oxalates, etc. of polyvalent metals, and, as the polyvalent metal, Zn, Fe, Mn, Ni, Co, Ca, Mg, Ba, Al and Sn are

preferred also in the aspect of the industrial cost, and Zn is further preferred among them. As preferred specific examples of the inorganic polyvalent metal compound, there can be mentioned zinc phosphate, zinc oxide, iron zinc phosphate, iron phosphate (ferrous phosphate, ferric phosphate), iron oxalate, manganese phosphate, nickel phosphate, cobalt phosphate, calcium phosphate, calcium hydrogenphosphate, calcium oxide, calcium hydroxide, etc., and among them zinc phosphate and zinc oxide are particularly preferably used.

The particle size of the inorganic polyvalent metal compound is preferably as small as possible for making the coated particles of lubricant use, and, specifically, is preferably 300  $\mu\text{m}$  or less and more preferably 100  $\mu\text{m}$  or less. As to the lower limit, there is no particular limitation, but from a limitation on preparation, the order of 0.3  $\mu\text{m}$  is usually a limit. When it is intended to obtain the coated particles of the invention in a state suspended in water, the average particle size of the inorganic polyvalent metal compound is preferably 20  $\mu\text{m}$  or less, and more preferably 10  $\mu\text{m}$  or less. When the average particle size is more than 20  $\mu\text{m}$ , it gets difficult to maintain stably the state dispersed in water.

The metallic soap coating the inorganic polyvalent metal compound in the invention is a salt between the polyvalent metal and the fatty acid composing the alkali soap or the like, the salt being formed by reaction of the inorganic polyvalent metal compound with the alkali soap or the like. As the metallic soap, there can be mentioned salts between a polyvalent metal such as Zn, Fe, Mn, Ni, Co, Ca, Al or Sn and a saturated fatty acid or unsaturated fatty acid having preferably 8 to 22, more preferably 16 to 20 carbon atoms (for example, palmitic acid, stearic acid, eicosanoic acid, oleic acid, etc.), and zinc stearate is mentioned representatively.

From the viewpoint of sufficiently coating the surfaces of the nuclei, the proportion of the metallic soap coatings to all the coated particles is preferably 1 to 30% by mass, and more preferably 2 to 15% by mass.

The coated particles of the invention also include particles each of which consists of a particle consisting of two layers of an inorganic polyvalent metal compound and a metallic soap of the polyvalent metal coating the metal compound, and a coating of an alkali soap or the like coating the particle. In the particles consisting of these three layers, the particles each of which consists of the inorganic polyvalent metal compound and the metallic soap of the polyvalent metal coating it may be the same as those mentioned above. In the three-layer particles, the proportion of the coatings of the alkali soap or the like to all the particles is preferably 0.1 to 5% by mass, more preferably 0.1 to 3% by mass in view of minimizing the amount of water soluble ingredients for the purpose of heightening the heat resistance of the particles and maintaining stable lubricating properties.

In the invention, the alkali soap or the like is not only needed for preparing the two-layer particles, but itself forms the outmost layer of the three-layer particles. The alkali soap or the like used in the invention is an alkali metal salt, ammonium salt or water soluble ester of a fatty acid. As the fatty acid, saturated fatty acids or unsaturated fatty acids having 8 to 22, particularly 16 to 20 carbon atoms are preferred, and there can specifically mentioned octanoic acid, decanoic acid, lauric acid, myristic acid, palmitic acid, stearic acid, eicosanoic acid, oleic acid, etc. As the alkali metal, sodium, potassium and lithium are preferred. As the water soluble ester, there can be mentioned an ester obtained by ring-opening polymerizing ethylene oxide to the carboxyl group of the above fatty acid, etc. As preferred specific examples of the alkali soap or the like, there can be mentioned a sodium or potassium salt of palmitic acid, stearic acid or eicosanoic

acid, and most preferred among them is sodium stearate. Sodium stearate may include both pure one and one containing sodium salts of other fatty acids. As the latter sodium stearate, sodium stearate put on the market as C18 soap is mentioned, and its composition is 95% or more of sodium stearate, less than 3% of C<sub>16</sub> fatty acids and less than 1% of mixed C<sub>15</sub> and C<sub>17</sub> fatty acids.

The present invention also relates to powder consisting of the above coated particles (namely, the above two-layer particles or three-layer particles).

The present invention also relates to a suspension wherein the above two-layer particles are suspended in water or an aqueous solution of an alkali soap or the like, the average particle size of the particles of the inorganic polyvalent metal compound being 20  $\mu\text{m}$  or less. The average particle size of the particles of the inorganic polyvalent metal compound in the two-layer particles is preferably 10  $\mu\text{m}$  or less. When the average particle size is more than 20  $\mu\text{m}$ , it gets difficult to maintain the water suspension state stably. The proportion of metallic soap coatings to all the two-layer particles in the suspension is preferably 1 to 30% by mass, more preferably 2 to 15% by mass, as is the case of the above-mentioned two-layer particles. It is possible to compound into the suspension a surfactant, a dispersant, a water soluble resin or the like in view of further heightening the stability of the dispersoid. The proportion of the two-layer particles to the whole suspension is not particularly limited so long as stable suspension of the two-layer particles is maintained, but, usually, is preferably on the order of 1 to 50% by mass, more preferably on the order of 5 to 40% by mass.

Description is made below on processes for preparation of the above powder and suspension of the invention.

The powder of the invention can be obtained by suspending particles of the above inorganic polyvalent metal compound in an aqueous solution of an alkali soap or the like, stirring the resulting suspension under heating to form metallic soap coating on the surfaces of the particles of the inorganic polyvalent metal compound, and drying the suspension.

As to use amount of the alkali soap or the like to the inorganic polyvalent metal compound, the alkali soap or the like may be used so that the above-mentioned proportion of the metallic soap to the coated particles may be obtained, but, specifically, it is preferred that the mole ratio of the inorganic polyvalent metal compound:the alkali soap or the like is the range of 100:0.05 to 100:25. When the amount of the alkali soap or the like is less than 100:0.05, the amount of the metallic soap layer gets extremely small, and expected effect tends not to be exerted sufficiently. When the amount of the alkali soap or the like is more than 100:25, the efficiency of the coating reaction is extremely reduced to bring about economical disadvantage. When the powder of the invention is used in lubricant use, the mole ratio of the inorganic polyvalent metal compound:the alkali soap or the like is preferably in the range of 100:0.25 to 100:15. When the amount of the alkali soap or the like is less than 100:0.25, sufficient lubrication performance tends hard to obtain, and it is more than 100:15, such problems tend to occur that the foaming properties of the suspension gets high due to existence of a lot of unreacted alkali soap or the like, and so on.

For accelerating reaction in preparation of the powder, it is preferred to adjust the temperature of the suspension to 60°C. or more, particularly 70 to 100°C., and the pH to 9 or more, particularly 10 to 12. As to the mechanism of the reaction, it is presumed that, on particles of the inorganic polyvalent metal compound, double decomposition reaction between the inorganic polyvalent metal compound and the alkali soap or the like takes place, and metallic soap layers coat the particles

## 11

of the inorganic polyvalent metal compound as nuclei. For making the pH the above-mentioned alkali side, there can be used hydroxides (sodium hydroxide, potassium hydroxide, etc.), carbonates (sodium carbonate, potassium carbonate, etc.), bicarbonates (sodium bicarbonate, potassium bicarbonate, etc.) of alkali metal, aqueous ammonia, etc., and preferred among them is sodium hydroxide. After surfaces of the particles of the inorganic polyvalent metal compound are coated with a preferred amount of metallic soap coatings, the suspension is dried into powder, and the method of the drying may be a conventional one. For example, a method of filtering the suspension and drying the resulting solid, a method of spray drying the suspension, or the like can be adopted.

Powder obtained by the above-mentioned process for preparing the powder of the invention is, usually, powder of three-layer particles consisting of the inorganic polyvalent metal compound, the metallic soap and the alkali soap or the like. Powder of two-layer particles consisting of the inorganic polyvalent metal compound and the metallic soap can be prepared by washing away the alkali soap or the like composing the outermost layer of the three-layer particles obtained in a way as mentioned above, with hot water, aqueous alcohol solution or the like.

The suspension of the invention can be obtained by suspending particles of the inorganic polyvalent metal compound in an aqueous solution of an alkali soap or the like, and stirring the suspension under heating to form metallic soap coating on the surfaces of the particles of the inorganic polyvalent metal compound. In this case, for suspending the particles of the inorganic polyvalent metal compound stably, the particle size of the particles of the inorganic polyvalent metal compound needs to be adjusted to 20  $\mu\text{m}$  or less, and is preferably adjusted to 10  $\mu\text{m}$  or less. For further stabilizing the suspension state, it is possible to compound a surfactant, a dispersant, a water soluble resin or the like.

The use amount of the alkali soap or the like to the inorganic polyvalent metal compound, the temperature and pH of the suspension for accelerating the reaction, and additives for making the pH the above-mentioned alkaline side may be the same as in the case of the preparation of the powder of the invention.

The powder and suspension relating to the metallic soap of the invention exert excellent performance as lubricants used in the cold plastic working field, etc. Namely, coating formed by making the powder or suspension of the invention adhering to the surface of a material to be subjected to cold plastic working shows excellent performance as lubricating coating for cold plastic working. When the powder of suspension is used for forming lubricating coating, the powder or suspension alone can be made into coating, but it can also be made into coating together with other general ingredients such as lubricating waxes, solid lubricants, extremely pressure additives, coating forming resins and/or viscosity adjusting agents. For example, by using the powder or suspension together with a lubricating oil containing a mineral oil or palm oil as a main ingredient, or a olefin wax or high molecular wax which melts and is liquidized at the time of working, it is possible to give the latter (i.e., the lubricating oil, etc.) excellent seizure resistance.

When the powder or suspension of the invention is compounded into a lubricating coating to give it seizure resistance, the compounding is preferably made so that the content of the powder or the solid matter in the suspension in the resulting coating may be 1% by mass or more, particularly 5% by mass or more. When the compounding proportion of the powder or the solid matter in the suspension is less than 1% by mass, it is impossible to give the lubricating coating

## 12

sufficient seizure resistance. Although the conditions for the adhesion are not particularly limited, the dry coating thickness of the lubricating coating is preferably made to be in the range of 0.5 to 50  $\mu\text{m}$ , more preferably made to be in the range of 1.0 to 30  $\mu\text{m}$ . When the coating thickness is less than 0.5  $\mu\text{m}$ , there is an anxiety that, especially in the strong working field, sufficient seizure resistance cannot be obtained to cause poor working. Further, the coating thickness of more than 50  $\mu\text{m}$  is superfluous and only increases the amount of the coating peeling away at introduction into the tool, and, thus, tends to bring about economical disadvantage.

A method for forming, on the surface of a material to be wrought, lubricating coating containing the powder or solid matter in the suspension of the invention is not particularly limited, and a conventional method can be adopted. For example, in the case of the aqueous suspension, lubricating coating can be obtained by making the aqueous suspension adhere onto the surface of the material by immersion treatment, spraying, roll coater treatment or the like, and then drying the resulting wet coating by natural seasoning, compulsory hot air drying or the like. In this operation, it is possible to mix a resin, an inorganic salt or the like for heightening the adhesion of the powder or the solid matter in the suspension, or an oil, a soap, a metallic soap, a wax or the like for supplementing the lubricity of powder or the solid matter in the suspension.

Further, as to a method for forming coating solely from the powder in a dry state, the powder of the invention can be made to adhere by a powder box method, an electrostatic coating method or the like, and an electrostatic coating method is particularly preferred because control of adhesion properties and adhesion amount is easy and stable and uniform lubricating coating can be obtained. It is also possible to mix a resin ingredient or wax ingredient having a low melting point, when the powder is made to adhere, for preventing peeling of the powder from the surface of the material to be wrought, and then heat the material to be wrought to immobilize the powder. It is also possible to mix powder of soap, metallic soap, wax, resin or the like for supplement of lubricity. Further, it is possible to obtain lubricating coating of a continuous coating state, through working heat and pressure, by, after making the powder of the invention adhere, subjecting the material to be wrought to light plastic working of the order of skin pass; and the operation is preferred since the resulting coating is coating further excellent in lubrication performance and barrier performance such as corrosion resistance. Particularly, lubricating coating obtained by a combination of electrostatic coating method and light plastic working of the order of skin pass is equal to "coating of phosphating treatment plus soap treatment" in all performance aspects. In this occasion, coating obtained after mixing the powder with a high molecular synthetic wax in a ratio by mass of preferably 1:9 to 9:1, more preferably 1:1 to 9:1 is excellent in lubricity, oil resistance, etc.

#### Detailed Description Particularly on the Invention as a More Practical Applied Invention

The invention is described in detail below. The particles of the invention each of which consists of a polyvalent metal salt of phosphoric acid as a nucleus and a metallic soap of the polyvalent metal coating the nucleus, namely particles of coated polyvalent metal salt of phosphoric acid give the resulting coating heat resistance and lubricity. It is necessary for a polyvalent metal salt of phosphoric acid to be selected to be sparingly soluble or insoluble in water. As preferred examples of the polyvalent metal in the polyvalent metal salt

of phosphoric acid, there can be mentioned Zn, Fe, Mn, Ni, Co, Ca, Mg, Ba, Al and Sn, and further preferred among them are Zn, Fe and Ca. As specific examples of the polyvalent metal salt of phosphoric acid, there can be mentioned zinc phosphate, iron zinc phosphate, iron phosphate (ferrous phosphate, ferric phosphate), manganese phosphate, nickel phosphate, cobalt phosphate, calcium phosphate, calcium hydrogenphosphate, magnesium phosphate, magnesium hydrogenphosphate, aluminum phosphate, tin phosphate, etc., and preferred among them are zinc phosphate, iron zinc phosphate, iron phosphate (ferrous phosphate, ferric phosphate), calcium phosphate and calcium hydrogenphosphate. These can be used alone or in combination of two or more.

The particles of the coated polyvalent metal salt of phosphoric acid exist in coating obtained by applying the lubricating coating forming agent of the invention onto a metallic material to be subjected to cold plastic working, and give the metallic material seizure resistance and lubricity; and, after being introduced into a die by melted coating ingredients at the time of working, exert an action to repair coating defects, namely a self-repairing action. For these purposes, in a state suspended in water or an aqueous solution of an alkali soap or the like, the average particle size of the particles of the coated polyvalent metal salt of phosphoric acid is preferably 30  $\mu\text{m}$  or less, more preferably 0.3 to 30  $\mu\text{m}$  and still more preferably 0.5 to 20  $\mu\text{m}$ . The average particle size of the polyvalent metal salt of phosphoric acid in the particles of the coated polyvalent metal salt of phosphoric acid is preferably 20  $\mu\text{m}$  or less, more preferably 0.2 to 20  $\mu\text{m}$  and still more preferably 0.4 to 10  $\mu\text{m}$ . Furthermore, for giving sufficient lubricity, the proportion by mass of the metallic soap coatings to all the particles of the coated polyvalent metal salt of phosphoric acid is preferably 1 to 30%, more preferably 2 to 15%.

The particles of the coated polyvalent metal salt of phosphoric acid are included in "two-layer particles" in the present invention particularly as a fundamental invention, and can be prepared in a similar way as in the two-layer particles.

Next, the water soluble inorganic salt needs to have not only a property to give the lubricating coating hardness but also a property to immobilize the particles of the coated polyvalent metal salt of phosphoric acid in the coating. A water soluble inorganic salt selected therefor needs to have a property to dissolve in water uniformly and, when the solution is applied onto a metallic material and dried, form firm coating. It is preferred to use, as the water soluble inorganic salt having such properties, at least one selected from the group consisting of alkali metal salts of sulfuric acid, alkali metal salts of silicic acid and alkali metal salts of boric acid. As specific examples thereof, there can be mentioned sodium sulfate, potassium sulfate, sodium silicate, potassium silicate, sodium borate, potassium borate, etc., and these can be used alone or in combination of two or more.

The water soluble organic acid salt needs to have a property not only to give hardness to the lubricating coating, but to immobilize the particles of the coated polyvalent metal salt of phosphoric acid in the coating. A water soluble organic acid salt selected therefor needs to have a property to dissolve in water uniformly and, when the solution is applied onto a metallic material and dried, form firm coating. It is preferred to use, as the water soluble organic acid salt having such properties, at least one selected from the group consisting of alkali metal salts of malic acid, alkali metal salts of succinic acid, alkali metal salts of citric acid and alkali metal salts of tartaric acid. As more specific examples thereof, there can be mentioned sodium malate, potassium malate, sodium succi-

nate, potassium succinate, sodium citrate, potassium citrate, sodium tartrate, potassium tartrate, etc.

The compounding proportion between the particles of the coated polyvalent metal salt of phosphoric acid (A) and the total of the water soluble inorganic salt and the water soluble organic acid salt (B) as a ratio by mass in solid matter of (B)/(A) is preferably 0.01 to 20.0, more preferably 0.01 to 16.0 and still more preferably 0.01 to 7.5. At less than 0.01, the particles of the coated polyvalent metal salt of phosphoric acid are not immobilized in the coating, the water soluble inorganic salt of the lubricating coating is not drawn into the tool against shear onto the coating at the time of working, and seizure resistance gets insufficient. On the other hand, at more than 20.0, since a probability that the water soluble inorganic salt having a high friction coefficient exists on the coating surface gets extremely high, the friction coefficient of the coating gets high, the coating gets easy to break and seizure gets liable to occur.

The lubricating coating forming agent of the invention may contain a smectite clay mineral according to necessity, and it is usually preferred to incorporate it. The smectite clay mineral used in the invention is a clay mineral having the following general formula. ("Clay Handbook 2nd edition" edited by Japan Clay Society and published by Gihodo Publishing CO., Ltd., pages 58-66, 1987):  $X_m(Y^{2+}, Y^{3+})_{2-3}Z_4O_{10}(OH)_2\cdot nH_2O$  wherein X is at least one of K, Na,  $\frac{1}{2}$  Ca and  $\frac{1}{2}$  Mg, m is 0.25 to 0.6,  $Y^{2+}$  is at least one of  $Mg^{2+}$ ,  $Fe^{2+}$ ,  $Mn^{2+}$ ,  $Ni^{2+}$ ,  $Zn^{2+}$  and  $Li^{+}$ ,  $Y^{3+}$  is at least one of  $Al^{3+}$ ,  $Fe^{3+}$ ,  $Mn^{3+}$  and  $Cr^{3+}$ , Z is at least one of Si and Al, and  $nH_2O$  is water among layers.  $Y^{2+}$ ,  $Y^{3+}$  in  $(Y^{2+}, Y^{3+})$  means  $Y^{2+}$  and/or  $Y^{3+}$ . Further, in the above, X represents a cation among the layers, Y is a cation of the octahedron and Z is a cation of the tetrahedron.

The smectite clay mineral used in the invention needs to have a property to give dispersion stability in liquid to the particles of the coated polyvalent metal salt of phosphoric acid and stabilize distribution of the particles in the coating. Therefor, formation of stable sol in an aqueous phase and increase of viscosity accompanying sharp increase of the concentrations of the contained ingredients get necessary. Smectite clay minerals generally show the above-mentioned properties when dispersed in an aqueous phase, and as smectite clay minerals having such properties, it is preferred to use at least one selected from the group consisting of hectorite, montmorillonite, beidellite, nontronite, saponite, iron saponite, stevensite and sauconite. Smectite clay minerals can be obtained not only as natural resources but as synthetic ones, and both can be used in the invention.

The compounding proportion of the smectite clay mineral as a ratio by mass in terms of solid matter of (C)/(A) wherein (A) are the particles of the coated polyvalent metal salt of phosphoric acid and (C) is the smectite clay mineral is preferably 0.005 to 0.5, more preferably 0.01 to 0.4. At less than 0.005, an effect to improve the dispersion stability of the particles of the coated polyvalent metal salt of phosphoric acid in the liquid and an effect to stabilize the distribution in the coating are not sufficient, and at more than 0.5, the lubricating coating forming agent gets a paste state to make its stable use difficult.

The lubricating coating forming agent of the invention may contain an auxiliary lubricant according to necessity, and, usually, it is preferred to incorporate it in the agent. The auxiliary lubricant needs to have an action to lower the friction coefficient of lubricating coating formed by the lubricating coating forming agent of the invention, and, as a melt carrier introducing the particles of the coated polyvalent metal salt of phosphoric acid between the material to be wrought and the tool, help the self-repairing effect of the

coating. Therefor, the auxiliary lubricant, as one which melts with heat generated at the time of plastic working to give the coating slipping properties and acts as a melt carrier, is preferably at least one selected from the group consisting of oil, soap, metallic soap, wax and polytetrafluoroethylene. As the oil, there can be used vegetable oils, synthetic oils, mineral oils, etc., and there can, for example, be mentioned palm oil, castor oil, rapeseed oil, machine oil, turbine oil, spindle oil, ester oil, silicone oil, etc. The soap is an alkali metal salt of a fatty acid, and there can, for example, be mentioned sodium salts, potassium salts, etc. of saturated or unsaturated fatty acids having 8 to 22 carbon atoms such as octanoic acid, decanoic acid, lauric acid, myristic acid, palmitic acid, stearic acid, eicosanoic acid and oleic acid. As the metallic soap, there can be mentioned salts of polyvalent metals such as calcium, zinc, magnesium and barium with the above-mentioned fatty acids. As the wax, there can be mentioned polyethylene wax, polypropylene wax, carnauba wax, paraffin wax, etc. As the polytetrafluoroethylene, there can be mentioned polytetrafluoroethylene having a molecular weight of the order of 1,000,000 to 10,000,000. It is preferred that such an auxiliary lubricant is incorporated in the lubricating coating forming agent by mixing it in the form of aqueous emulsion or aqueous dispersion with other ingredients. The auxiliary lubricant is usually dispersed or emulsified in the lubricating coating forming agent of the invention.

The compounding proportion of the auxiliary lubricant as a ratio by mass in terms of solid matter of (D)/(A) wherein (A) are the particles of the coated polyvalent metal salt of phosphoric acid and (D) is the auxiliary lubricant is preferably 0.03 to 18.0, more preferably 0.05 to 15.0 and still more preferably 0.5 to 5.0. At less than 0.03, the friction coefficient of the lubricating coating is increased and the effect to act as a melt carrier is not sufficient, and at more than 18.0, the coating is softened, and the coating tends to be broken because it gets incapable of withstanding shearing force thereon at the time of working.

The lubricating coating forming agent of the invention may contain an organic high molecular compound according to necessity. It is preferred that the organic high molecular compound is water soluble or water dispersible and has a weight average molecular weight of 1,000 to 1,000,000. The organic high molecular compound needs to have an action to give coating strength to lubricating coating formed using the lubricating coating forming agent. The organic high molecular compound is not particularly limited so long as it has coating formability, and there can, for example, be mentioned resin as a polymer of ethylenically unsaturated monomer(s) (particularly, acrylic resin), urethane resin, epoxy resin, phenol resin, hydroxymethylcellulose, carboxymethylcellulose, etc. It is preferred that such an organic high molecular compound is incorporated in the lubricating coating forming agent by mixing it in the form of aqueous emulsion or aqueous dispersion with other ingredients. In view of improving the coating strength of coating formed by the lubricating coating forming agent, the organic high molecular compound is added into the lubricating coating forming agent so that its content can be preferably 0.5 to 25% by mass, more preferably 1.0 to 15% by mass based on the whole solid matter including itself.

In plastic working wherein the working is severe, it is possible to further incorporate a solid lubricant in the lubricating coating forming agent. As the solid lubricant in such a case, one existing stably in the coating and capable of assisting lubrication at a high load is preferred. As such solid lubricants, there can be mentioned graphite, molybdenum disulfide, boron nitride, fluorinated graphite, mica, etc.

In plastic working wherein the working is severer, it is possible to incorporate an extremely pressure additive in the lubricating coating forming agent. As the extremely pressure additive in such a case, one existing stably in the coating and capable of exerting extreme-pressure effect at the contact surface between the tool and the metal is preferred. As such extremely pressure additives, there can be mentioned sulfur containing extremely pressure additives, organomolybdenum extremely pressure additives, phosphorus containing extremely pressure additives and chlorine containing extremely pressure additives such as sulfurized olefins, sulfurized esters, sulfites, thiocarbonates, chlorinated fatty acids, phosphoric esters, phosphorous esters, molybdenum dithiocarbamate (MoDTC), molybdenum dithiophosphate (MoDTP) and zinc dithiophosphate (ZnDTP).

When a dispersant is necessary to disperse or emulsify the particles of the coated polyvalent metal salt of phosphoric acid, the auxiliary lubricant, and/or the solid lubricant and/or extremely pressure additives, as such a dispersant, there can be used a dispersant selected from nonionic surfactants, anionic surfactants, amphoteric surfactants, cationic surfactants, water soluble high molecular dispersants and so on.

There is no particular limitation on a process for preparing the lubricating coating forming agent of the invention so long as a lubricating coating forming agent prepared meets the above-mentioned conditions. For example, the agent can be obtained by adding particles of a coated polyvalent metal salt of phosphoric acid, and, as optional ingredients, a smectite clay mineral, an auxiliary lubricant, and/or a solid lubricant and/or an extremely pressure additive, if necessary after being made into a dispersion or emulsion using a dispersant and water, into an aqueous solution of a water soluble inorganic salt and/or a water soluble organic acid salt; and then stirring the resulting mixture. The solid matter concentration of the lubricating coating forming agent is not particularly limited so long as the lubricating coating forming agent prepared meets the above-mentioned conditions, but, in view of handling properties and stability of the lubricating coating forming agent, the solid matter concentration is preferably 1 to 80% by mass, more preferably 10 to 60% by mass.

The lubricating coating forming agent of the invention can be used as a lubricant used when a metallic material such as iron or steel, stainless steel, plated steel (for example, steel subjected to plating treatment such as electrogalvanizing, molten zinc plating, aluminum zinc plating, aluminum plating or iron zinc plating), aluminum or aluminum alloy, magnesium alloy, tin or tin alloy, titanium or titanium alloy, or copper or copper alloy is subjected to cold plastic working such as forging, wire drawing, tube reducing or sheet forming. There is no particular limitation on the shape of the metallic material.

For exerting good lubricity, it is preferred, prior to applying the lubricating coating forming agent of the invention, to pretreat a metallic material to be worked in order of cleaning (usually, an alkali cleaner is used), water washing, descaling (shot blasting or acid washing with hydrochloric acid or the like) and water washing to clean the surface of the metallic material. When oxidation scale does not adhere or the metallic material is used in a use where oxidation scale is needed, descaling and succeeding water washing can be omitted. These pretreatments can be carried out by conventional ways.

The lubricating coating forming agent of the invention is applied to the surface of a metallic material by a conventional method such as immersion, spraying or *流しあげ*. The application is carried out until the metal surface is sufficiently coated with the lubricating coating forming agent, and there is no particular limitation on time of the application. After the

application, the lubricating coating forming agent needs to be dried. The drying may be made by allowing the coating to stand at ordinary temperature, but, usually, is preferably made at 60 to 150° C. for 10 to 60 minutes. In view of preventing seizure, the coating mass of the lubricating coating forming agent is preferably 1 g/m<sup>2</sup> or more, more preferably 3 to 30 g/m<sup>2</sup>.

Lubricating coating obtained from the lubricating coating forming agent of the invention shows stable cold plastic working performance because the particles of the coated polyvalent metal salt of phosphoric acid having good seizure resistance and slipping properties are uniformly held in the coating by immobilizing effect of the water soluble inorganic salt and/or the water soluble organic acid salt, and the smectite clay mineral. Furthermore, since, because the auxiliary lubricant ingredient melting by heat generation due to working acts as a melt carrier, and so on, the particles of the coated polyvalent metal salt of phosphoric acid are drawn into the die and exert a self-repairing action on coating defect parts, the lubricating coating shows stable lubricity, even in tube drawing working such as tube reducing or wire drawing wherein lubricating coating forming treatment is, usually, carried out in such a state such as a banded state or a coiled state that the resulting coating is liable to be ununiform.

### EXAMPLES

The present invention is further specifically described below together with its effects, by giving examples of the invention together with comparative examples.

#### I. Examples and Comparative Examples on the Invention as a Fundamental Invention

##### 1. Preparation of Suspension and Powder of Metallic Soap-Coated Particles

A suspension and powder of metallic soap-coated particles were prepared according to the processes shown below. For confirming that coated particles, wherein nuclei of the inorganic polyvalent metal compound are coated with coatings of the metallic soap, are prepared, soap ingredients in the powder prepared or soap ingredients in the powder obtained by drying the suspension prepared were separated into alkali soap or the like dissolving in an aqueous ethanol solution and metallic soap not dissolving therein, and the mass of each was measured, whereby

formation of metallic soap was confirmed. The above method is explained in more detail below. One gram of a powder sample was stirred in aqueous 50% ethanol solution for 4 hours, and the mixture was filtered with filter paper. Then, the filtrate and the residue were heated in 1N hydrochloric acid, respectively, to decompose the soap ingredients into fatty acid(s). Each of the mixtures was extracted with diethyl ether, and the proportion of metallic soap formation=([(fatty acid(s) from the metallic soap)/(fatty acid(s) from the alkali soap or the like+fatty acid(s) from the metallic soap)]×100) was calculated. When the proportion of metallic soap formation is 50% or more, it was judged that the nuclei surfaces were coated with a sufficient amount of metallic soap layers.

###### (A1)

Ten grams of sodium stearate and 1 g of sodium hydroxide were mixed with 100 g of particles of zinc phosphate having an average particle size of 1 μm and dispersed in 1 L of water, and the mixture was stirred at a liquid temperature of 90 to 95° C. for 30 minutes to obtain a suspension of metallic soap-coated particles.

•X: Proportion of metallic soap formation=82% (this value corresponds to about 8% as the proportion by mass of metallic soap coatings based on all the two-layer particles)

###### 5 (A2)

Two hundred grams of zinc phosphate powder, 30 g of potassium stearate and 1 g of potassium hydroxide were dispersed into 700 mL of water under stirring, and the mixture was stirred at a liquid temperature of 70° C. for 1 hour. Solid matter was recovered by filtration, and stirred for 4 hours in aqueous 50% ethanol solution, and, by second filtration, solid matter was obtained. This was dried in an oven of 100° C. to obtain dry powder of metallic soap-coated particles containing no layer of the alkali soap.

•X: Proportion of metallic soap formation=78% (this value corresponds to about 10% as the proportion by mass of metallic soap coatings based on all the two-layer particles).

###### 10 (A3)

Two hundred grams of zinc oxide, 10 g of sodium stearate and 3 g of sodium hydroxide were dispersed into 700 mL of water under stirring, and the mixture was stirred at a liquid temperature of 90° C. for 20 minutes. Then, solid matter was recovered by filtration and dried in an oven of 100° C. to obtain dry powder of metallic soap-coated particles.

•X: Proportion of metallic soap formation=53% (this value corresponds to about 3% as the proportion by mass of metallic soap coatings based on all the three-layer particles)

###### 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 98

TABLE 1

| Sample powder  | Results of resistance to oil pollution |
|----------------|----------------------------------------|
| Example I-1    | A2                                     |
| Example I-1    | A3                                     |
| Com. exam. I-1 | B3                                     |
| Com. exam. I-2 | B6                                     |

Note:

Com. exam.: Comparative example

### 3. Evaluation as Lubricating Coating Forming Material

The compositions of the lubricating coatings of Examples I-3 to I-9 obtained by using, as lubricating coating forming materials, the suspension of the metallic soap-coated particles of the invention prepared in the above or the powders of the metallic soap-coated particles of the invention prepared in the above, and the compositions of the lubricating coatings of Comparative examples I-3 to I-7 not using suspension of metallic soap-coated particles nor powder of metallic soap-coated particles of the present invention are shown in Table 2.

#### 3.1. Lubricating Coating Forming Material

Lubricating coating forming materials used in the present test are shown below.

- (A1) The suspension of the metallic soap-coated particles of the invention obtained in the above
- (A2) The powder of the metallic soap-coated particles of the invention obtained in the above
- (A3) The powder of the metallic soap-coated particles of the invention obtained in the above
- (A4) Aqueous suspension of zinc phosphate particles having an average particle size of 0.5  $\mu\text{m}$
- (A5) Zinc oxide powder having an average particle size of 50  $\mu\text{m}$
- (B1) Water-dispersed polyethylene wax
- (B2) Water-dispersed olefin wax
- (B3) Calcium stearate powder
- (B4) Montanic acid wax powder
- (B5) Oxidized polyethylene wax powder
- (B6) Zinc stearate powder
- (C1) Sodium polyacrylate (molecular weight 10,000)
- (C2) Aqueous emulsion of urethane resin (polyester urethane resin)

#### 3.2. Treating Method

For forming lubricating coating of an example of the invention or a comparative example on the surface of a test material, one of the following treating methods was used.

##### (a) Immersion Treatment Method

A test piece whose surface was cleaned was immersed in lubricating coating forming suspension of ordinary temperature to make the suspension adhere thereon, and was subjected to drying in a hot air drying furnace of 100° C. to form

lubricating coating on the surface of the test piece. The amount of the dry coating adhering was about 15 g/m<sup>2</sup>.

##### (b) Electrostatic Coating Method

A test piece whose surface was cleaned was electrostatically coated with lubricating coating forming powder to form lubricating coating in a powder adhesion state on the surface of the test piece. As an electrostatic powdering apparatus, GX300 made by Nihon Parkerizing Co., Ltd was used, and the lubricating coating forming powder was charged at a voltage of 60 kV. Adhesion of the charged lubricating coating forming powder on the surface of the test piece by an electrostatic coating method was carried out using an electrostatic coating gun GX116 made by Nihon Parkerizing Co., Ltd. Air pressures for supply of the powder in this operation were 98 kPa as the main air pressure and 196 kPa as the sub-air pressure. The coating time was 1 second, and the amount of the powder coating adhering was about 15 g/m<sup>2</sup>.

#### 3.3. Test Method and Evaluation Criterion

##### 3.3.1. Spike Test

Spike test working was made according to the method disclosed in JP 5-7969 A, and lubricity was evaluated by the spike height of the test piece after the working. The higher the spike height is, the better the lubricity is.

Test piece: A material used for the test was annealed S45C material which was made spherical and commercially available, and the shape of the test piece was 25 mm  $\phi$  in diameter and 30 mm in height.

Evaluation criterion: A: Spike height was 13 mm or more  
 B: Spike height was 12 mm or more but less than 13 mm  
 C: Spike height was less than 12 mm  
 D: The material was seized onto the die, resulting in molding being impossible

##### 3.3.2. Drawing Test

Steel wire as a test piece coated with a lubricating coating was subjected to drawing working of the order of skin pass (first drawing: reduction in area being 10.3%), and, then, subjected to drawing working of reduction in area being 31.5% (second drawing), using a draw bench drawing testing machine on the market.

Test piece: A material used for the test was SCr440 material on the market, and the shape of the test piece was 9.5 mm  $\phi$  in diameter and 1 m in length.

Evaluation criterion:

- A: Seizure and flaws were not found up to the second drawing
- B: Seizure was not found up to the second drawing, but some flaws were found.
- C: Seizure and flaws were not found up to the first drawing, but seizure occurred at the second drawing resulting in drawing being impossible
- D: Seizure occurred at the first drawing resulting in drawing being impossible

TABLE 2

| Composition of lubricating film |                                                        |                                                |                                            |                 |
|---------------------------------|--------------------------------------------------------|------------------------------------------------|--------------------------------------------|-----------------|
|                                 | Seizure resisting ingredient<br>(compounding amount %) | Lubricant ingredient<br>(compounding amount %) | Other ingredient<br>(compounding amount %) | Treating method |
| Example                         | I-3 A1 (100)                                           | —                                              | —                                          | a               |
|                                 | I-4 A1 (50)                                            | B1 (45)                                        | C1 (5)                                     | a               |
|                                 | I-5 A1 (20)                                            | B2 (70)                                        | C2 (10)                                    | a               |
|                                 | I-6 A2 (100)                                           | —                                              | —                                          | b               |

TABLE 2-continued

| Composition of lubricating film |                                                        |                                                |                                            |                    |
|---------------------------------|--------------------------------------------------------|------------------------------------------------|--------------------------------------------|--------------------|
|                                 | Seizure resisting ingredient<br>(compounding amount %) | Lubricant ingredient<br>(compounding amount %) | Other ingredient<br>(compounding amount %) | Treating<br>method |
| Com. exam                       | I-7 A2 (80)                                            | B4 (20)                                        | —                                          | b                  |
|                                 | I-8 A3 (50)                                            | B5 (50)                                        | —                                          | b                  |
|                                 | I-9 A3 (30)                                            | B4 (60)                                        | C1 (10)                                    | b                  |
|                                 | I-3 A4 (100)                                           | —                                              | —                                          | a                  |
|                                 | I-4 A4 (50)                                            | B1 (45)                                        | C1 (5)                                     | a                  |
|                                 | I-5 A5 (100)                                           | —                                              | —                                          | b                  |
|                                 | I-6 A5 (50)                                            | B3 (50)                                        | —                                          | b                  |
|                                 | I-7 A5 (30)                                            | B5 (70)                                        | —                                          | b                  |

Note:

The compounding amount of each ingredient is compounding amount as solid matter

Com. exam.: Comparative example

TABLE 3

| Results of evaluation<br>as lubricating film<br>forming material |            |            |              |
|------------------------------------------------------------------|------------|------------|--------------|
|                                                                  |            | Spike test | Drawing test |
| Example                                                          | I-3        | B          | B            |
|                                                                  | I-4        | A          | A            |
|                                                                  | I-5        | A          | A            |
|                                                                  | I-6        | B          | B            |
|                                                                  | I-7        | A          | A            |
|                                                                  | I-8        | B          | B            |
|                                                                  | I-9        | A          | B            |
|                                                                  | Com. exam. | D          | D            |
|                                                                  | I-4        | C          | C            |
|                                                                  | I-5        | D          | D            |
|                                                                  | I-6        | C          | D            |
|                                                                  | I-7        | C          | C            |

Note:

Com. exam.: Comparative example

As shown in the above results of evaluation (see Table 3), each of the lubricating coatings of Examples I-3 to I-9 obtained by using the metallic soap compositions of the invention which play a role of seizure resisting ingredient and, at the same time, also have lubricating performance, showed good lubricating performance. On the other hand, in Comparative examples I-3 to I-7, because of exposure of the seizure resisting ingredient having high friction coefficient, the resulting lubricating coatings could not exert sufficient performance as lubricating coating being subjected to strong working, and, moreover, load to the tool is judged to be high.

As apparent from the above explanation, the coated particles of the invention consisting of an inorganic polyvalent metal compound as a nucleus, and metallic soap coating or metallic soap coating plus coating of alkali soap or the like on it coating the nucleus, are mainly used as ingredients for coating type lubricating coating, and are suitable as materials which are excellent in seizure resistance, and, because of their low surface friction coefficient, can inhibit wear of tools at the time of plastic working, and do not easily cause pollution of working oil. Therefore, the industrial utility value of the present invention is extremely great.

II. Examples and Comparative Examples on the  
Invention as a Particularly Practical Applied  
Invention

Examples II-1 to II-12 and Comparative Examples  
II-1 to II-9

Lubricating coating forming agents of ingredients and their compositions shown in Table 4 were prepared.

<Coating of Polyvalent Metal Salt of Phosphoric Acid With Metallic Soap>

As to Examples II-1 to II-12 and Comparative examples II-1, II-2, II-5 and II-6, coating of a polyvalent metal salt of phosphoric acid [ingredient (A)] with metallic soap was carried out (Table 4). Specifically, 90 g of a polyvalent metal salt of phosphoric acid having an average particle size of 1 to 5  $\mu\text{m}$  dispersed in 1 L of water, 9 g of sodium stearate and 1 g of potassium hydroxide were mixed and stirred at a liquid temperature of 80 to 85°C. for 30 minutes to obtain a suspension of particles of coated polyvalent metal salt of phosphoric acid.

<Preparation of the Lubricating Coating Forming Agent of Example II-1>

Preparation of a lubricating coating forming agent was made so that the respective ingredients got to be the ratios of Table 4. The procedure of the preparation is as follows. First, the water soluble inorganic salt was dissolved in water, and then the smectite clay mineral was incorporated in the solution and uniformly dispersed. Thereafter, the above suspension of particles of coated polyvalent metal salt of phosphoric acid was incorporated in the suspension, and then the auxiliary lubricant was added, and the mixture was stirred to prepare the lubricating coating forming agent of Example II-1.

As to starting materials used in Example II-1, the polyvalent metal salt of phosphoric acid is zinc phosphate (solid), the water soluble inorganic salt is aqueous 50% by mass sodium silicate dispersion, and the smectite clay mineral is montmorillonite (solid).

The lubricating coating forming agents of Examples II-2 to II-12 and Comparative examples II-1 to II-7 were prepared in the similar manner as above. The lubricating coating forming agents of Comparative example II-8 is an existing coating type lubricating coating forming agent, and the lubricating coating forming agent of Comparative example II-9 is a phosphate salt plus soap treating agent on the market.

## &lt;Test Piece&gt;

The following test pieces were used for the following evaluations.

Friction coefficient measuring test: SPCC-SB 150 mm×70 mm×0.8 mm (t is thickness)

Evaluation of forging properties: S45C annealed material which was made spherical 30 mm φ×18 to 40 mm

Tube reducing properties: STKM17A 25.4 mm φ×2.5 mm×2,000 mm

Wire drawing properties: S45C annealed material 3.0 mm φ×50,000 mm

## &lt;Coating Forming Treatment&gt;

coating forming treatment was made according to the following steps.

In the Cases of Examples II-1 to II-12 and Comparative Example II-1 to II-8

(1) Cleaning: a degreasing agent on the market (registered trademark Fine Cleaner 4360, made by Nihon Parkerizing Co., Ltd.), concentration 20 g/L, temperature 60° C., immersion 10 minutes

(2) Water washing: tap water, room temperature, immersion 30 seconds

(3) Descaling: hydrochloric acid washing, concentration 17.5%, room temperature, immersion 10 minutes

(4) Water washing: tap water, room temperature, immersion 30 seconds

(5) Treatment: treating agent of an example or comparative example, room temperature, immersion 10 seconds, targeted adhesion amount 5g/m<sup>2</sup>

(6) Drying: 80° C., 5 minutes

In the Case of Comparative Example II-9

(1) Cleaning: a degreasing agent on the market (registered trademark Finecleaner 4360, made by Nihon Parkerizing Co., Ltd.), concentration 20 g/L, temperature 60° C., immersion 10 minutes

(2) Water washing: tap water, room temperature, immersion 30 seconds

(3) Descaling: hydrochloric acid washing, concentration 17.5%, room temperature, immersion 10 minutes

(4) Water washing: tap water, room temperature, immersion 30 seconds

(5) Chemical conversion coating treatment: Zinc phosphate chemical conversion coating agent on the market (registered trademark Palbond 181X, made by Nihon Parkerizing Co., Ltd.), concentration 90 g/L, temperature 80° C., immersion 10 minutes

(6) Water washing: tap water, room temperature, immersion 30 seconds

(7) Soap treatment: reactive soap lubricant on the market (registered trademark Palube 235, made by Nihon Parkerizing Co., Ltd.), concentration 70 g/L, temperature 80° C., immersion 5 minutes

(8) Drying: 80° C., 3 minutes

## &lt;Coating Performance Evaluation Test&gt;

A friction coefficient measurement test was made, after the above coating forming treatment, according to a Bowden test which is the most standard friction coefficient measurement test. Since, in the Bowden test, there is a stable stage of friction coefficient after initial sliding, the friction coefficient at the stable stage was regarded as the friction coefficient of the lubricating coating. Measurement conditions in the test are as follows.

Sliding type: reciprocating sliding type

Steel sphere: 10 mmφSUJ2 steel sphere

Vertical load: 50N

Sliding velocity: 10 mm/s

Temperature: 60° C.

Sliding number of times: 200 times

A forging test was made by a backward piercing test. The backward piercing test is such a test that cylindrical test pieces are subjected to backward piercing working wherein punches are knocked into the test pieces, the heights of the test pieces are varied from 18 mm up to 40 mm by every 2 millimeters, and possible working degree is determined.

When seizure resistance is insufficient, flaws due to seizure are formed on the internal surfaces of the test pieces and on the punches. These flaws were checked by visual observation, and the highest height of the test pieces where no flaw is formed was evaluated as showing the lubricity of a lubricating

coating forming agent. The treatment was carried out both by a method of treating test pieces separately one by one (one piece treatment) and by a method of treating plural pieces together in a rotary barrel (barrel treatment). Evaluation criterion is shown below. A and B are practical levels.

20 A: The workable height of the test piece is 40 mm or more.  
B: The workable height of the test piece is 36 mm or more, but less than 40 mm.

C: The workable height of the test piece is 32 mm or more, but less than 36 mm.

25 D: The workable height of the test piece is less than 32 mm.

A tube reducing test was made by carrying out tube reducing working under the following conditions and making evaluation by such limiting reduction in area that no seizure was formed. The limiting reduction in area was assumed to be such reduction in area that three pipes were subjected to the tube reducing working and all the three pipes could be worked. The treatment was carried out both by a method of treating pipes separately one by one (one pipe treatment) and by a method of treating three pipes in a bundled state (bundle treatment). Evaluation criterion is shown below. A and B are practical levels.

Die: R die

Plug: cylindrical plug.

30 Tube reducing velocity: 15 m/min.

A: The limiting reduction in area is 50% or more.  
B: The limiting reduction in area is 43% or more, but less than 50%.

C: The limiting reduction in area is 38% or more, but less than 43%.

45 D: The limiting reduction in area is less than 38%.

A wire drawing test was made by carrying out wire drawing working under the following conditions and making evaluation by such limiting wire drawing velocity that stable wire drawing was possible. The coating treatment was carried out both by a method of extremely loosening the bundled state of the wire rod coil so that the wire rods could not contact mutually (a method of stretching the coil into a spring state; one rod treatment) and by a method of treating the wire rod coil in a bundled state so as to promote contact among the wire rods (bundled treatment). Evaluation criterion is shown below. A and B are practical levels.

Die: R die; 2.75 mm φ

50 Reduction in area: 15.0%

Wire drawing velocity: 10 to 100 m/min.

A: Limiting wire drawing velocity is 100 m/min or more.  
B: Limiting wire drawing velocity is 80 m/min or more, but less than 100 m/min.

C: Limiting wire drawing velocity is 60 m/min or more, but less than 80 m/min.

D: Limiting wire drawing velocity is less than 60 m/min.

## &lt;Test Results&gt;

Results of the above tests are shown in Table 5. As apparent from Table 5, the lubricating coating forming agents of the invention in Examples II-1 to II-12 showed good lubricity irrespective of working forms, and also showed stable lubricity even in the cases of barrel treatment and bundled treatment where uniform treatment was difficult. On the other hand, the lubricating coating forming agents of Comparative examples II-1 and II-2 which contain metallic soap-coated particles but no water soluble inorganic salt nor water soluble organic acid salt showed only low lubricity even when they were applied uniformly. Further, in Comparative examples II-3 and II-4 where the surfaces of particles of the polyvalent metal salt of phosphoric acid were not coated with metallic soap, since the friction coefficients of the particles were high and the self-repairing effect of the resulting coatings was not exerted, lubricity was not stable in the barrel treatment and the bundled treatment. The lubricating coating forming agents of Comparative examples II-5 and II-6 where calcium hydroxide or iron oxalate poor in solubility in water was used in place

of a water soluble inorganic salt or a water soluble organic acid salt could not form continuous coating, and the resulting coatings are low in lubricity. In Comparative examples II-7 and II-8 where particles of a coated polyvalent metal salt of phosphoric acid are not contained, since the self-repairing effect of the resulting coatings was not exerted, lubricity was not stable in the barrel treatment and the bundled treatment. In the phosphating treatment plus soap treatment of Comparative example II-9, stable lubricity was exerted irrespective of treating methods, but loads to the environment are large in view of treatment of industrial wastes and waste water, control of treating liquids, high energy consumption by high temperature treatment, and so on. Thus, the lubricating coating forming agent of the invention, because of containing particles of a coated polyvalent metal salt of phosphoric acid and a water soluble inorganic salt, can prevent lowering of lubricity owing to ununiform coating which was the most difficult problem of coating-type lubricating coating forming agent, and can realize stable lubricity.

TABLE 4

| Examples II-1 to II-12 and Comparative examples II-1 to II-9 |                                                      |                                             |                 |                  |                               |          |           |
|--------------------------------------------------------------|------------------------------------------------------|---------------------------------------------|-----------------|------------------|-------------------------------|----------|-----------|
|                                                              | Ingredient *1                                        |                                             |                 |                  | Ratio by mass as solid matter |          |           |
|                                                              | (A)                                                  | (B)                                         | (C)             | (D)              | (B)/(A)                       | (C)/(A)  | (D)/(A)   |
| Example (II)                                                 | 1 zinc phosphate                                     | sodium silicate*2                           | montmorillonite | —                | 10.0                          | 0.01     | —         |
|                                                              | 2 zinc phosphate                                     | potassium silicate*3                        | hectorite       | paraffin wax     | 2.0                           | 0.05     | 1.5       |
|                                                              | 3 zinc phosphate                                     | potassium tetraborate                       | —               | polyethylene wax | 0.02                          | —        | 15.0      |
|                                                              | 4 zinc iron phosphate                                | sodium silicate*2                           | hectorite       | sodium stearate  | 0.5                           | 0.25     | 0.5       |
|                                                              | 5 zinc iron phosphate                                | sodium citrate                              | —               | machine oil      | 0.01                          | 0.005    | 1.0       |
|                                                              | 6 zinc iron phosphate                                | sodium sulfate                              | nonttronite     | —                | 1.0                           | 0.5      | —         |
|                                                              | 7 iron phosphate                                     | sodium silicate +<br>potassium sulfate*4    | —               | palm oil         | 16.0                          | —        | 2.0       |
|                                                              | 8 iron phosphate                                     | sodium tetraborate                          | hectorite       | paraffin wax     | 0.5                           | 0.01     | 0.5       |
|                                                              | 9 iron phosphate                                     | potassium sulfate +<br>potassium silicate*5 | sauconite       | paraffin wax     | 3.5                           | 0.05     | 2.0       |
|                                                              | 10 calcium phosphate                                 | sodium silicate*2                           | nonttronite     | —                | 10.0                          | 0.3      | —         |
| Comparative example (II)                                     | 11 calcium phosphate                                 | potassium sulfate +<br>potassium silicate*4 | —               | polyethylene wax | 15.0                          | —        | 0.05      |
|                                                              | 12 calcium phosphate                                 | sodium sulfate                              | hectorite       | palm oil         | 7.5                           | 0.4      | 2.0       |
|                                                              | 1 zinc phosphate                                     | —                                           | —               | calcium stearate | —                             | 0.2      | 2.5       |
|                                                              | 2 zinc iron phosphate                                | —                                           | nonttronite     | polyethylene wax | —                             | 0.1      | 12.0      |
|                                                              | 3 zinc phosphate*6                                   | sodium silicate*2                           | nonttronite     | —                | 0.1                           | 0.05     | —         |
|                                                              | 4 calcium phosphate*6                                | sodium tetraborate                          | —               | palm oil         | 5.0                           | —        | 5.0       |
|                                                              | 5 iron phosphate                                     | calcium hydroxide                           | —               | paraffin wax     | 2.0                           | —        | 2.5       |
|                                                              | 6 zinc iron phosphate                                | iron oxalate                                | —               | polyethylene wax | 1.0                           | —        | 0.5       |
|                                                              | 7 —                                                  | potassium silicate*7                        | —               | graphite*8       | —                             | *9       | —         |
| Proportion of ingredient as solid matter*10                  |                                                      |                                             |                 |                  |                               |          |           |
|                                                              |                                                      |                                             |                 |                  | (B)                           | (D)      | (E)       |
| 8                                                            | Existing coating-type lubricating film forming agent |                                             |                 |                  | 35%                           | 50%      | 15%       |
| Adhesion mass (g/m <sup>2</sup> )                            |                                                      |                                             |                 |                  |                               |          |           |
|                                                              |                                                      |                                             |                 |                  | phosphate                     | metallic | unreacted |
|                                                              |                                                      |                                             |                 |                  | salt                          | soap     | soap      |
| 9                                                            | Phosphate salt treatment + soap treatment            |                                             |                 |                  | 6.7                           | 2.3      | 3.2       |

Notes of Table 4

\*1 As to ingredients, (A) is a polyvalent metal salt of phosphoric acid, (B) is a water soluble inorganic salt or water soluble organic acid salt, (C) is a smectite clay mineral, and (D) is an auxiliary lubricant.

\*2SiO<sub>2</sub>:Na<sub>2</sub>O = 2:1\*3SiO<sub>2</sub>:K<sub>2</sub>O = 3:1

\*4Sodium sulfate:sodium metasilicate = 7:3

\*5Sodium sulfate:potassium silicate (SiO<sub>2</sub>:K<sub>2</sub>O = 3:1) = 7:3

\*6Zinc phosphate and calcium phosphate whose surfaces are not coated with coating of metallic soap of these polyvalent metals were used.

\*7SiO<sub>2</sub>:K<sub>2</sub>O = 4:1

\*8In place of an auxiliary lubricant, graphite was used as a solid lubricant.

TABLE 4-continued

| Examples II-1 to II-12 and Comparative examples II-1 to II-9 |  |     |  |     |  |     |  | Ratio by mass as solid matter |         |         |
|--------------------------------------------------------------|--|-----|--|-----|--|-----|--|-------------------------------|---------|---------|
| Ingredient *1                                                |  |     |  |     |  |     |  |                               |         |         |
| (A)                                                          |  | (B) |  | (C) |  | (D) |  | (B)/(A)                       | (C)/(A) | (D)/(A) |

\*9 Comparative example 7 was carried out using potassium silicate ( $\text{SiO}_2\text{:K}_2\text{O} = 4:1$ ):graphite = 6:4.

\*10 In Comparative example 8, Ingredient B is sodium tetraborate, Ingredient D is calcium stearate, and Ingredient E is urethane resin (made by Dai-ichi Kogyo Seiyaku Co., Ltd.; Superflex 110).

\*11 Furthermore, as Ingredient (E), a phenol resin (made by Gunei Kagaku Co., Ltd.; Resitop PL-6020) was used in Example 9, and an urethane resin (made by Dai-ichi Kogyo Seiyaku Co., Ltd.; Superflex 110) in Example 12. The phenol resin and the urethane resin were used in amounts of 7.0% by mass and 8.5% by mass, respectively, based on the total of Ingredients (A) to (E), in terms of solid matter.

TABLE 5

| Results of evaluation (Examples II-1 to II-12 and Comparative examples II-1 to II-9) |                       |        |                          |        |                         |        |                     |        |     |             |
|--------------------------------------------------------------------------------------|-----------------------|--------|--------------------------|--------|-------------------------|--------|---------------------|--------|-----|-------------|
| Friction coefficient                                                                 | Results of evaluation |        |                          |        |                         |        |                     |        |     |             |
|                                                                                      | Forging properties    |        | Tube reducing properties |        | Wire drawing properties |        | Load to environment |        |     |             |
|                                                                                      | one                   | barrel | one                      | banded | one                     | banded | one                 | banded | one | environment |
| Example (II)                                                                         | 1                     | 0.07   | A                        | A      | B                       | B      | B                   | B      | ○   |             |
|                                                                                      | 2                     | 0.06   | A                        | A      | A                       | A      | A                   | A      | ○   |             |
|                                                                                      | 3                     | 0.05   | A                        | B      | B                       | B      | B                   | B      | ○   |             |
|                                                                                      | 4                     | 0.06   | A                        | A      | A                       | A      | A                   | A      | ○   |             |
|                                                                                      | 5                     | 0.05   | B                        | B      | B                       | B      | B                   | B      | ○   |             |
|                                                                                      | 6                     | 0.07   | B                        | B      | B                       | B      | B                   | B      | ○   |             |
|                                                                                      | 7                     | 0.07   | A                        | B      | A                       | B      | A                   | B      | ○   |             |
|                                                                                      | 8                     | 0.06   | A                        | A      | A                       | A      | A                   | A      | ○   |             |
|                                                                                      | 9                     | 0.06   | A                        | A      | A                       | A      | A                   | A      | ○   |             |
|                                                                                      | 10                    | 0.07   | B                        | B      | B                       | B      | B                   | B      | ○   |             |
|                                                                                      | 11                    | 0.06   | A                        | B      | A                       | B      | A                   | B      | ○   |             |
|                                                                                      | 12                    | 0.06   | A                        | A      | A                       | A      | A                   | A      | ○   |             |
| Comparative examples (II)                                                            | 1                     | 0.06   | C                        | D      | C                       | D      | B                   | D      | ○   |             |
|                                                                                      | 2                     | 0.05   | C                        | C      | C                       | C      | B                   | B      | ○   |             |
|                                                                                      | 3                     | 0.10   | D                        | D      | D                       | D      | D                   | D      | ○   |             |
|                                                                                      | 4                     | 0.08   | B                        | C      | B                       | D      | B                   | C      | ○   |             |
|                                                                                      | 5                     | 0.08   | B                        | D      | B                       | D      | B                   | C      | ○   |             |
|                                                                                      | 6                     | 0.06   | B                        | D      | B                       | D      | B                   | C      | ○   |             |
|                                                                                      | 7                     | 0.07   | C                        | D      | C                       | D      | C                   | C      | ○   |             |
|                                                                                      | 8                     | 0.07   | B                        | D      | B                       | D      | B                   | C      | ○   |             |
|                                                                                      | 9                     | 0.06   | B                        | B      | A                       | A      | A                   | A      | X   |             |

Lubricating coatings obtained by applying the lubricating coating forming agent of the invention onto the surfaces of various metallic materials give the metallic materials excellent cold plastic working properties, namely excellent lubricity and excellent seizure resistance. Particularly, the lubricating coating forming agent of the invention can give metallic materials excellent working performance even in barrel treatment and bundled treatment where it has been difficult for conventional coating-type lubricating coating forming agent to give stable working performance.

The invention claimed is:

1. A process for cold plastic working of metallic materials which comprises

forming on the surface of a metallic material a lubricating coating containing, in an amount of 1% by mass or more, particles each of which particles consists of a water sparingly soluble or water insoluble polyvalent metal salt of phosphoric acid as a nucleus and a coating of a metallic soap of the polyvalent metal coating the surface of the nucleus, the polyvalent metal being at least one metal selected from Zn, Fe, Mn, Ni, Co, Mg, Ba, Al and Sn, the metallic soap being formed by reaction of the polyvalent metal salt of phosphoric acid with an alkali metal salt, ammonium salt or water soluble ester of a fatty acid, said particles being hereinafter called two-

45

50

55

60

65

layer particles, or particles each of which consists of each of the two-layer particles and a coating of an alkali metal salt, ammonium salt or water soluble ester of a fatty acid coating the surface of the two-layer particle, said particles being hereinafter called three-layer particles, and

subjecting the resulting metallic material to cold plastic working.

2. The process according to claim 1 wherein the particles are two-layer particles, the average particle size of the polyvalent metal salt of phosphoric acid is 300  $\mu\text{m}$  or less and the proportion of all the metallic soap coatings to all the two-layer particles is 1 to 30% by mass.

3. The process according to claim 1 wherein the polyvalent metal salt of phosphoric acid is zinc phosphate.

4. The process according to claim 1 wherein the particles are three-layer

particles, the average particle size of the polyvalent metal salt of phosphoric acid is 300  $\mu\text{m}$  or less, the proportion of all the metallic soap coatings to all the two-layer particles is 1 to 30% by mass, and the proportion of all the coatings of the alkali metal salt, ammonium salt or water soluble ester of the fatty acid to all the three-layer particles is 0.1 to 5% by mass.

29

5. The process according to claim 1 wherein the formation of the lubricating coating is carried out by making powder consisting of the two-layer particles or the three-layer particles, or a mixture of the powder with at least one additive selected from the group consisting of waxes; solid lubricants, extremely pressure additives, coating forming resins, viscosity adjusting agents, lubricating oils, soaps and metallic soaps, then adhered to the surface of a metallic material.

6. The process according to claim 5 wherein, the additive is at least one additive selected from the group consisting of waxes, coating forming resins, soaps and metallic soaps, and after the powder or the mixture of the powder with the additive which is adhered onto the surface of the metallic material, the resulting metallic material is subjected to light plastic working of the order of skin pass, and then, subjecting the resulting metallic material to cold plastic working.

7. The process according to claim 1 wherein the formation of the lubricating coating is carried out by making a suspension wherein the two-layer particles are suspended in water or an aqueous solution of an alkali metal salt, ammonium salt or water soluble ester of a fatty acid, the average particle size of particles of the polyvalent metal salt of phosphoric acid being 20  $\mu\text{m}$  or less, and the proportion of all the metallic soap coatings to all the two-layer particles being 1 to 30% by mass, adhering the coating onto the surface of the metallic material, and then, drying the resulting coating.

8. The process according to claim 7 wherein the suspension contains at least one additive selected from the group consisting of waxes, solid lubricants, extremely pressure additives, coating forming resins, viscosity adjusting agents, lubricating oils, soaps and metallic soaps.

9. The process according to claim 1 wherein dry coating thickness of the lubricating coating is 0.5 to 50  $\mu\text{m}$ .

10. A process for cold plastic working of metallic materials which comprises

applying onto the surface of a metallic material a lubricating coating forming agent wherein particles each of which consists of a water sparingly soluble or water insoluble polyvalent metal salt of phosphoric acid as a nucleus and a coating of a metallic soap of the polyvalent metal coating the surface of the nucleus, said particles being hereinafter referred to as particles of coated polyvalent metal salt of phosphoric acid, are suspended in an aqueous solution of a water soluble inorganic salt and/or a water soluble organic acid salt; the polyvalent metal being at least one selected from Zn, Fe, Mn, Ni, Co, Mg, Ba, Al and Sn, the metallic soap being formed by reaction of the polyvalent metal salt of phosphoric acid with an alkali metal salt, ammonium salt or water soluble ester of a fatty acid, and each of the water soluble inorganic salt and organic acid salt having a property to form a firm coating when it is uniformly dissolved in water and the resulting solution is applied onto a metallic material and dried;

30

drying the resulting wet coating to form a lubricating coating; and then, subjecting the resulting metallic material to cold plastic working.

5 11. The process according to claim 10 wherein the polyvalent metal salt of phosphoric acid is at least one selected from zinc phosphate, zinc iron phosphate and iron phosphate.

12. The process according to claim 10 wherein the average particle size of the particles of coated polyvalent metal salt of phosphoric acid is 30  $\mu\text{m}$  or less, and the average particle size of the polyvalent metal salt of phosphoric acid is 20  $\mu\text{m}$  or less.

13. The process according to claim 10 wherein the proportion of all the metallic soap coatings to all the particles of coated polyvalent metal salt of phosphoric acid is 1 to 30% by mass.

14. The process according to claim 10 wherein the water soluble inorganic salt is at least one selected from an alkali metal salt of sulfuric acid, an alkali metal salt of silicic acid and an alkali metal salt of boric acid.

20 15. The process according to claim 10 wherein the water soluble organic acid salt is at least one selected from an alkali metal salt of malic acid, an alkali metal salt of succinic acid, an alkali metal salt of citric acid and an alkali metal salt of tartaric acid.

25 16. The process according to claim 10 wherein the proportion by mass of the total of the water soluble inorganic salt and the water soluble organic acid salt (B) to the particles of coated polyvalent metal salt of phosphoric acid (A), namely (B)/(A), in terms of solid matter, is within the range of 0.01 to 20.0.

17. The process according to claim 10 wherein the lubricating coating forming agent contains a smectite clay mineral in such an amount that the proportion by mass of the smectite clay mineral (C) to the particles of coated polyvalent metal salt of phosphoric acid (A), namely (C)/(A), in terms of solid matter, is within the range of 0.005 to 0.5.

30 18. The process according to claim 10 wherein the lubricating coating forming agent contains, as an auxiliary lubricating ingredient, at least one auxiliary lubricating ingredient (D) selected from an oil, a soap, a metallic soap, a wax and polytetrafluoroethylene in such an amount that the proportion by mass of the auxiliary lubricating ingredient (D) to the particles of coated polyvalent metal salt of phosphoric acid (A), namely (D)/(A), in terms of solid matter, is within the range of 0.03 to 18.0.

45 19. The process according to claim 10 wherein the lubricating coating forming agent contains a water soluble or water dispersible organic macromolecular compound having a weight average molecular weight of 1,000 to 1,000,000 in such an amount that its content in the resulting coating gets to be within 0.5 to 25% by mass based on the whole dry coating.

\* \* \* \* \*